

## 1

3,644,510

### PROPYLENE OXIDATION IN THE PRESENCE OF IRIDIUM METAL

Noel W. Cant and William K. Hall, Pittsburgh, Pa., as-  
signors to Gulf Research & Development Company,  
Pittsburgh, Pa.

No Drawing. Filed Nov. 25, 1968, Ser. No. 778,805

Int. Cl. C07c 53/08

U.S. Cl. 260—533 R

8 Claims

#### ABSTRACT OF THE DISCLOSURE

Propylene is oxidized with oxygen to acetic acid, acro-  
lein, etc. by oxidation in the contact presence of iridium  
metal.

This invention relates to a process for oxidizing pro-  
pylene to obtain a useful mixture of organic compounds  
comprising acetic acid, acrolein and acetone.

In addition to the above desired compounds, by-pro-  
ducts such as carbon dioxide and water are also formed.  
It was expected that the partial oxidation of propylene  
would yield primarily organic acids containing three car-  
bon atoms, i.e. propionic acid. Quite unexpectedly, it has  
been found that the main product of the oxidation reaction  
is acetic acid so long as the oxidation reaction is car-  
ried out in the presence of iridium metal.

In accordance with the invention, therefore, propylene  
is oxidized to a product comprising acetic acid by reacting  
propylene with a gas containing free molecular oxygen in  
the contact presence of iridium metal.

In order to obtain good selectivity to the desired oxy-  
genated compounds it is important that the propylene  
together with a gas containing free molecular oxygen be  
contacted with the iridium metal either supported or un-  
supported at a temperature within the range of about  
50° C. to about 300° C., and preferably within the range  
of about 80° C. to about 200° C. Since the reaction is  
exothermic, means must be provided to control the tem-  
perature of the reaction within the limits defined above.  
Below the lower temperature limits defined above the re-  
action rate becomes too low to be economically feasible,  
whereas at temperatures above the upper limits, the yield  
of desired oxygenated compounds decreases with the con-  
current production of excessive amounts of water and  
carbon dioxide. The temperature can be controlled by  
any suitable means, and one method of at least partially  
controlling the temperature is to dilute the iridium metal  
by distending it on a suitable support material such as  
silica, magnesia, alumina, thoria or mixtures thereof. The  
iridium metal can, of course, be used unsupported and  
when this is done the metal can be in any suitable form,  
such as sponge form. When the iridium is distended on a  
support, the surface area of the support is not critical and  
can suitably be between 0.1 and 600 square meters per  
gram. In addition to the above named supports, mate-  
rials such as carbon, kiesulguhr, pumice, the natural clays,  
mullite and alundum are also suitable. When the iridium  
metal is supported, suitable amounts of iridium metal are  
from 0.2 to 30 weight percent of the total catalyst with  
preferred amounts from one of ten weight percent and the  
more preferred amounts from one to five weight percent  
of the total catalyst.

The method of preparing the supported or unsupported  
catalysts is not critical. Suitable methods of preparing the  
supported catalysts, for example, include the method of  
incipient wetness using aqueous solutions of suitable iri-  
dium salts such as  $H_2IrCl_6$  followed by drying and reduc-  
tion in hydrogen to obtain the metal.

## 2

Another method of controlling the temperature is to  
dilute the propylene-oxygen mixture with an inert gas  
such as nitrogen or helium. Yet another method of con-  
trolling the reaction temperature is to pass the admixture  
of propylene and oxygen over the iridium metal catalyst  
at very high space velocities. Suitable gaseous space veloc-  
ities are within the range of about one to about 2000 vol-  
umes of propylene measured at standard temperature and  
pressure per volume of catalyst per hour, and the pre-  
ferred space velocities are from about five to about 200.

A total operating pressure of about one atmosphere is  
the desired operating pressure. Higher or lower pressures  
can be used; for example, pressures of from 0.5 to 15  
atmospheres or more can suitably be employed.

The ratio of the partial pressure of oxygen to the  
partial pressure of propylene can suitably be between 0.2  
and 100 and is preferably between two and 30. The partial  
pressure of propylene should be at least 0.05 p.s.i.a.  
and is preferably from 0.1 to one p.s.i.a. when the total  
pressure is atmospheric (14 p.s.i.a.). Correspondingly  
higher partial pressures of propylene would be employed  
at correspondingly higher total operating pressures.

The propylene is oxidized in the presence of a gas  
containing free molecular oxygen. Pure oxygen can be  
used, but this creates problems of temperature control as  
noted above. It is preferred that the free molecular oxygen  
be diluted with an inert gas such as nitrogen or helium.  
The volume percent of free molecular oxygen in the gas  
containing it can suitably be between one and 100 and is  
preferably between one and 20. When propylene is mixed  
with this gas containing free molecular oxygen, the par-  
tial pressure of oxygen is usually between 0.5 and ten  
p.s.i.a. and is preferably between two and five p.s.i.a. If  
the partial pressure of oxygen is below about 2.0 pounds  
per square inch absolute, selectivity to the desired oxy-  
genated products decreases, whereas above about two  
pounds per square inch absolute selectivity to the desired  
oxygenated compounds remains substantially constant.

The invention will be further described with reference  
to the following experimental work. In all of the exam-  
ples to follow the following procedure was employed. A  
single pass flow system was used wherein a feed mixture  
of propylene, oxygen and helium was passed through a  
bed (approximately two parts by volume of catalyst) of a  
supported iridium catalyst at a given temperature be-  
tween 50° C. and 200° C. at a flow rate of between 2400  
and 3000 volumes of total feed per hour. The contact time  
was about 2.3 seconds and the space velocity based on  
the total feed was about 1500 volumes of feed per volume  
of catalyst per hour. The propylene space velocities for  
any particular run can be calculated by multiplying 1500  
by the ratio of the propylene partial pressure in milli-  
meters to the total pressure of about 740 millimeters. The  
reaction products were cooled to —80° C. by indirect  
cooling to condense the reaction product which was most-  
ly acetic acid with minor amounts of acetone, acrolein,  
acrylic and/or propionic acids. Water and  $CO_2$  were  
formed as by-products.

#### EXAMPLE 1

In this run for this example, the feed mixture was  
passed through a bed of an alpha-alumina supported  
iridium catalyst containing 1.5 weight percent iridium.  
The results of this run are summarized in Table I below.

#### EXAMPLE 2

In the run for this example, the feed mixture was  
passed through a bed of a silica supported iridium  
catalyst containing five weight percent iridium. The silica  
support was a commercial Cab-O-Sil material obtained  
from the Cabot Company. The catalyst was prepared by

## 3

the method of incipient wetness by contacting the Cab-O-Sil with an aqueous solution of an appropriate amount of an iridium salt, i.e.  $H_2IrCl_6$ , drying the material and reducing at 300° C. in hydrogen to convert the salt to metallic iridium. The results of this run are summarized in Table I below.

Referring to Table I below, the percent selectivity to the useful oxygenated products was about the same (30.5 v. 28) for the alpha-alumina supported iridium catalyst (Example 1) as with the silica supported iridium catalyst (Example 2) at about the same oxidation rate.

A series of runs was made by passing a feed mixture containing varying amounts of oxygen, propylene and helium over the catalyst of Example 1 at varying conditions to determine the effect of changes in temperature and feed composition on reaction rate and selectivity to the production of acetic acid, acetone and acrolein. The results of this series of runs are given in Table II below.

Referring to Table II below, it can be seen that the selectivity to the production of acetic acid, acetone and acrolein decreases slightly in going from 100 to 123° C.

TABLE I.—PRODUCTS OF PROPYLENE OXIDATION OVER SUPPORTED IRIDIUM AT A TOTAL PRESSURE OF ABOUT 740 MM.

| Example No. | Metal | Support                        | Wt. percent metal | Oxygen pressure (mm.) | Propylene pressure (mm.) | Temp. (° C.) | Oxidation <sup>1</sup> Rate Volumes, $C_3H_6/min.$ | Percent selectivity <sup>2</sup> to— |                             |                       |      |
|-------------|-------|--------------------------------|-------------------|-----------------------|--------------------------|--------------|----------------------------------------------------|--------------------------------------|-----------------------------|-----------------------|------|
|             |       |                                |                   |                       |                          |              |                                                    | Acetic acid                          | Acrylic plus propionic acid | Acrolein plus acetone |      |
| 1.....      | Ir    | $\alpha\text{-Al}_2\text{O}_3$ | 1.5               | 131                   | 7                        | 135          | 0.16                                               | 25                                   | 0.5                         | 5.0                   | 30.5 |
| 2.....      | Ir    | $\text{SiO}_2$                 | 5.0               | 61                    | 21                       | 135          | 0.18                                               | 21                                   | 3                           | 4                     | 28   |

<sup>1</sup> The oxidation rate is defined as the rate at which propylene is converted to all products in volumes (STP) per minute, e.g. if the propylene is passed over the catalyst at two volumes per minute and it is found that 1.8 volumes per minute is recovered unchanged, then the oxidation rate is 2.0 minus 1.8, or 0.2 volumes per minute.

<sup>2</sup> The percent selectivity is defined as the percent of the propylene oxidized which is converted to the given product.

TABLE II.—DEPENDENCE OF RATE AND SELECTIVITY OF PROPYLENE OXIDATION OVER 1.5% Ir/ $\alpha\text{-Al}_2\text{O}_3$  ON PROCESS VARIABLES

| Ex. No. | Temp. (° C.) | Oxygen pressure (mm.) | Propylene pressure (mm.) | Oxidation rate <sup>a</sup> vols./min. | Percent selectivity <sup>a</sup> to— |         |          |
|---------|--------------|-----------------------|--------------------------|----------------------------------------|--------------------------------------|---------|----------|
|         |              |                       |                          |                                        | Acetic acid                          | Acetone | Acrolein |
| 3.....  | 101          | 42                    | 14                       | 0.04                                   | 15                                   | 1.3     | 0.2      |
| 4.....  | 105          | 41                    | 13                       | 0.06                                   | 14                                   | 1.9     | 0.3      |
| 5.....  | 110          | 43                    | 13                       | 0.09                                   | 13                                   | 1.8     | 0.2      |
| 6.....  | 116          | 41                    | 13                       | 0.12                                   | 13                                   | 1.7     | 0.1      |
| 7.....  | 123          | 39                    | 12                       | 0.22                                   | 11                                   | 1.6     | 0.1      |
| 8.....  | 132          | 40                    | 12                       | 0.41                                   | 9.5                                  | 1.2     | 0.1      |
| 9.....  | 105          | 53                    | 3                        | 0.016                                  | 18                                   | 2.5     | 1.0      |
| 10..... | 105          | 52                    | 6                        | 0.027                                  | 15                                   | 2.5     | 0.6      |
| 11..... | 105          | 52                    | 14                       | 0.042                                  | 14                                   | 1.9     | 0.3      |
| 12..... | 105          | 50                    | 21                       | 0.052                                  | 15                                   | 1.8     | 0.3      |
| 13..... | 105          | 54                    | 30                       | 0.053                                  | 13                                   | 1.5     | 0.2      |
| 14..... | 105          | 22                    | 13                       | 0.038                                  | 12                                   | 1.5     | 0.1      |
| 15..... | 105          | 47                    | 13                       | 0.041                                  | 15                                   | 1.7     | 0.3      |
| 16..... | 105          | 54                    | 14                       | 0.043                                  | 14                                   | 2.4     | 0.3      |
| 17..... | 105          | 89                    | 14                       | 0.028                                  | 19                                   | 1.7     | 0.4      |
| 18..... | 105          | 134                   | 14                       | 0.024                                  | 20                                   | 2.4     | 1.5      |

<sup>a</sup> See Table I footnotes.

(compare Examples 3-8). The rate, however, increases considerably with the increase in temperature (again compare Examples 3-8). The rate of oxidation increases with propylene pressure as can be seen by comparing Examples 9-13. The oxidation rate is not greatly affected by the oxygen partial pressure but the percent selectivity to useful oxygenated products increases with an increase in oxygen partial pressure as can be seen by a comparison of Runs 14-18.

Obviously, many modifications and variations of the invention as hereinabove can be made without departing from the spirit and the scope thereof, and such modifications and variations are intended to be included within the scope of this invention.

We claim:

1. A process for the production of a product comprising acetic acid, which process comprises reacting

## 4

propylene with a gas containing free molecular oxygen in the contact presence of iridium metal.

2. A process according to claim 1 wherein the reaction occurs at a temperature from 50° to 300° C., a partial pressure of oxygen above about 0.5 pounds per square inch absolute and a propylene space velocity from about one to about 2000.

3. The process of claim 2 wherein the temperature in the reaction zone is maintained in the range of about 80° to about 200° C.

4. A process according to claim 2 wherein the partial pressure of oxygen is within the range of about 0.5 to about 10 pounds per square inch absolute.

5. The process of claim 1 wherein the iridium metal is deposited on a support.

6. A process according to claim 5 wherein the reaction occurs at a temperature from 50° to 300° C. and the amount of iridium metal is from 0.2 to 30 weight percent of the total catalyst.

7. A process according to claim 6 wherein the support is alpha-alumina.

8. A process according to claim 6 wherein the support is silica.

## References Cited

## UNITED STATES PATENTS

3,439,044 4/1969 Hirsch et al. \_\_\_\_\_ 260—604  
3,534,093 10/1970 Gerberich et al. \_\_\_\_\_ 260—533 R

60 65 LORRAINE A. WEINBERGER, Primary Examiner

R. D. KELLY, Assistant Examiner

U.S. Cl. X.R.

70 260—597 B, 604 R